

July 17, 1951

H. VON FRAUNHOFER

2,561,299

COLOR CINEMATOGRAPHY

Filed March 7, 1946



INVENTOR

Hans von Fraunhofer

BY Pierce-Schaffler & Parker

ATTORNEYS

## UNITED STATES PATENT OFFICE

2,561,299

## COLOR CINEMATOGRAPHY

Hans von Fraunhofer, London, England

Application March 7, 1946, Serial No. 652,810  
In Great Britain July 23, 1945

1 Claim. (Cl. 95—2)

1

The various methods and processes for the production of colour motion pictures may be classified under two main groups, namely: (1) the "Additive" type systems and (2) the "Subtractive" type processes.

Although the additive type systems are capable of a remarkably close approximation to the appearance of nature, none is, unfortunately, free from fundamental limitations that prevent commercial adoption, nor is there any indication of the direction in which further improvements of a fundamental nature could be made in processes of this type.

The subtractive type processes, especially those of the multi-layer kind, because they represented the one branch of the art that gave some definite hope for future development and improvement, were finally adopted by the motion picture industry. Of these processes there are several which are giving quite satisfactory service today, but up to the present time, the manner of making of the required colour separation negatives remains complicated, and, in particular, the printing procedure is complicated and expensive. It is a known fact that the present processes of colour cinematography are not as simple as the black and white processes and, therefore, they are not suitable in cases, such as news-reel films, in which the elements of time and cost of production are of vital consideration.

My invention concerns a new process for materially simplifying colour motion picture procedure, from the making of the required colour separation negatives to the printing of the positives, and, in accordance with the invention, I combine the best features of the additive and subtractive principles of colour rendition without any of their known shortcomings.

Broadly, therefore, the invention may be said to consist in a process for the production of colour motion pictures wherein different frames of a negative film comprising two superimposed layers of emulsion are exposed through different colour filters in such manner as to effect a three-colour analysis, the two series of negative images are developed, differentially coloured and printed simultaneously on to two differently sensitised layers of emulsion comprised in a positive film, which are then developed and appropriately coloured, whereby in projection two of the component colours are obtained subtractively and the third component by an additive effect.

In carrying out the process I may employ a two-layer monopack or bipack film consisting of an orthochromatic and a panchromatic emulsion.

2

In accordance with my process, all of the red colour values are recorded in the usual uniform density on the panchromatic emulsion while the green and blue colour records are recorded on the orthochromatic emulsion in differential densities as compared between the odd and even frames throughout the entire length of the film.

In printing such two-layer monopack or bipack film on to a suitable double coated positive film, the result is two sets of alternate frames, namely, the red colour values of the one-layer in superimposition on the green colour values of the odd frames and in superimposition on the blue colour values of the even frames.

15 Further, this process proposes to use subtractive method of colouring the positives, by the conversion of the successive green and blue colour values of the one layer into an orange-red series of images and the red colour values of the other layer into a series of blue-green images by either dye-mordanting, chemical toning, colour development or by any other suitable means.

20 In accordance with the general theory upon which this process is designed to operate, the deep shadows and black are produced on the screen in the same manner as in the subtractive methods, that is, by the absorption of the light by means of the combination of the reduced silver deposits in the areas representing black in the two sets of images, namely, red and green and red and blue, while white on the other hand, is produced by the free transmission of light by the partial or complete absence of reduced silver deposits in the areas representing white in the two sets of images.

25 In accordance with the basic theory underlying this process, that is, by the slight variation of the silver deposit in one frame and layer from that in the next frame and layer, a differential colouring is given to the transmitted light alternately between the two sets of frames, and this produces, in projection, the required additive effect to obtain natural colours on the screen.

30 There are, obviously various ways in which an integral monopack or bipack negative film for this purpose may be produced without departing from the basic principle underlying this invention. However, the method I prefer for best results is as follows:

35 The integral monopack negative is formed by disposing on to the celluloid carrier a yellow dyed orthochromatic emulsion containing a dye forming substance of suitable type and character, as for instance p-nitrophenylacetoneitrile.

40 On to this blue and green sensitive emulsion

layer there is then coated or otherwise disposed a layer of a suitable minus green and blue dye, known to the art as a red-filter. This red-filter dye may be employed in a solution with gelatine or other suitable transparent material.

Finally, there is then coated on to the film a coating of red sensitive emulsion containing a dye forming substance of a suitable type and character, as for instance acetoacet 2,5 dichloroanilide.

The required slight variation of the silver deposit in one frame and layer from that in the next frame and layer to obtain the additive effect desired may be achieved by passing the film through a suitable machine which sprays, wipes, coats or otherwise deposits upon the Celluloid carrier a thin layer of suitable minus blue filter-dyes upon the odd frames of the film. Known examples of such minus blue filter-dyes are tartrazine, rapid filter yellow. Upon the adjacent even frames of the film a deposit of minus green filter-dye such as Rose bengal, rhodamine, is applied. Alternatively, there may be affixed to the camera, a suitable rotating disc arrangement containing the required filters, thus simplifying the manufacture of the integral monopack or bipack.

Obviously, monopack negatives formed in the above described manner must be exposed through the carrier, but by reversing the order and disposition of the two layers so that the emulsion containing the red sensitizer is nearest to the carrier and the blue-green emulsion furthest away from the carrier, exposure may be made in the usual manner with the emulsion facing the lens.

After exposure, the negative is developed in any suitable normal black and white developer and is then fixed and thoroughly washed. Thereafter the negative is bleached in a suitable bleach for dye coupling by re-development. Such bleach may be a mixture of one ounce (30.0 grams) of potassium ferricyanide, half an ounce (15.0 grams) of potassium bromide, and tap water to make 32 ounces (1 litre) of solution. The negative is bleached completely in this solution, then washed thoroughly and re-developed in a suitable coupling developer which may be composed as follows:

|                                    |       |      |
|------------------------------------|-------|------|
| Sodium sulphite                    | grams | 20.0 |
| Sodium carbonate                   | do    | 40.0 |
| Potassium bromide                  | do    | 2.0  |
| di-Ethyl-p-phenylenediamino hydro- |       |      |
| chloride                           | do    | .5   |

Water to make 1 litre

The result now is a coloured negative of which all of the red colour records of the top layer have been converted into a series of greenish-yellow images while the blue-green colour records of the lower layer have been turned into a series of magenta coloured images.

Obviously, the choice of the dye forming substance may be varied to obtain any suitable combination of colours for each of the two layers of images representing the blue-green and red colour records respectively.

Alternatively, instead of the use of dye forming substances in the emulsion, the two layers may be converted into colour by dye-mordanting, chemical toning or any other suitable process of which many are known to the art.

The primary purpose of converting the two series of images, incorporated in the two layers of emulsion of the negative, is to reduce the

printing of the positive into a single operation and thus to assure perfect registration of the two images and, therefore, to materially shorten the time of production.

5 My preferred method for making up of the required positive film is the following:

First a layer of orthochromatic emulsion containing an orange-red dye forming substance, such as for instance a suitable combination of 10 o - chloroacetoacetanilide and p - nitrophenyl-acetonitrile in the proportion of one-third and two-thirds respectively, is disposed upon the Celluloid carrier.

Thereafter, a yellow dyed blue sensitive emulsion containing a blue-green dye forming substance such as for instance 2,4 dichloro-1-naphthol is coated over the lower layer of the positive film.

The negative film described hereinbefore is 20 then printed in the usual black and white fashion by contact or optically, on to this special positive film after which the positive film receives substantially the same processing as that specified for the negative film. Reference may 25 be had to the accompanying drawing which indicates the course of the process by means of a briefed flow diagram.

It should be understood that the present disclosure is for the purpose of illustration only 30 and it will have been appreciated that regardless of whether an integral monopack or a bipack negative film is adopted for analysis purposes, or any double-coated film is used for printing of the positive, the same basic method 35 is employed, and, therefore, the colour images of the negative or of the positive print in each of the component two layers might be produced by any and every toning, mordanting or colour development or colour coupling process that has 40 ever been suggested or used without departing from the basic principle underlying this process and, therefore, all such modifications and equivalents fall within the scope of the invention. That is to say, that no matter what method 45 of processing may be used for the type of negative or positive material adopted, in one layer thereof the blue-green colour record of the negative will contain differential silver deposits in alternate frames of the positive and, in the other layer of the positive the red colour record printed from the negative will have a uniform deposit in all frames.

I claim:

55 A process for the production of colour motion pictures which give the effect of a three-colour analysis by means of a combination of additive and subtractive principles, said process comprising producing in a first layer of a two-layer negative film having a first light-sensitive emulsion layer of at least red sensitivity and a second light-sensitive emulsion layer of only orthochromatic sensitivity a series of consecutive frames each recording uniform density images 60 only of red colour values of a photographed subject, producing in said orthochromatic emulsion second layer of said two layer negative film a first series of alternate frames recording images from said subject only of blue-green colour values 65 of minus blue density and a second series of frames alternating with said first series recording images from said subject only of blue-green colour values of minus green density, converting the images in the frames of the series 70 of the first layer to greenish-yellow, converting 75 of the first layer to greenish-yellow, converting

the images in both series of the second layer to magenta, printing in a single operation by means of exposure through both layers of the thus coloured two-layer negative film both layers of a two-layer positive film having an orthochromatic-sensitive emulsion first layer protected by a yellow filter and a blue-sensitive emulsion second layer, colouring the images formed in the first layer of the positive orange-red, and colouring the images formed in the second layer of the positive blue-green.

HANS VON FRAUNHOFER.

6  
REFERENCES CITED  
The following references are of record in the file of this patent:

UNITED STATES PATENTS

| Number    | Name          | Date           |
|-----------|---------------|----------------|
| 1,278,162 | Kelley        | Sept. 10, 1918 |
| 1,954,452 | Mannes et al. | Apr. 10, 1934  |
| 1,966,653 | Thornton      | July 17, 1934  |
| 1,969,469 | Mannes et al. | Aug. 7, 1934   |
| 2,001,250 | Heymer        | May 14, 1935   |
| 2,059,884 | Mannes et al. | Nov. 3, 1936   |